

## UNITED STATES PATENT OFFICE

2,385,885

## DISCHARGE PRINTING OF CELLULOSE ACETATE

George W. Seymour and Victor S. Salvin, Cumberland, Md., assignors to Celanese Corporation of America, a corporation of Delaware

No Drawing. Application February 28, 1942,  
Serial No. 432,750

14 Claims. (Cl. 8—64)

This invention relates to improvements in the discharge printing of textile materials and relates more particularly to improvements in the discharge printing of fabrics made of or containing cellulose acetate, or other organic derivatives of cellulose, which have been dyed with azo dyestuffs.

An object of our invention is the discharge printing of textile materials and particularly fabrics made of or containing cellulose acetate or other organic derivative of cellulose which are dyed with certain azo dyes to obtain clear white discharge patterns.

Another object of our invention is the discharge printing of said dyed fabrics so as to obtain clear white discharge patterns as well as illuminated discharge patterns in but a single operation.

Other objects of our invention will appear from the following detailed description.

The discharge printing of textile materials is widely used in the dyeing art for obtaining pattern effects on fabrics in a simple and economical manner. Generally, the fabric which is to be printed is dyed in the piece in a solid color, by means of a suitable dyestuff, to provide the color desired as the background. When the fabric is dyed with an azo dyestuff, a chemically active discharge paste having a reducing action on the azo dye forming the background color is applied locally to the fabric in a predetermined pattern, and the fabric then treated so that the azo dye is reduced and the background color is removed at the points where the paste has been applied, yielding a pattern or design upon a colored background. The pattern should preferably have a clear white color. With many azo dyestuffs clear white discharges can not be obtained regardless of the discharging agent employed. In the case of fabrics dyed with some azo dyestuffs, however, clear white discharge patterns may be obtained, but only by employing certain discharging agents which are acid in reaction, such as, for example, zinc formaldehyde sulfoxylate. When attempts are made to discharge these azo dyes with discharge agents of alkaline reaction the pattern obtained after the application of the discharging agent is either spotted, or is of an off-shade of white, having a brownish, pinkish or other undesirable tint, depending upon the azo dye employed.

When it is desired to obtain a pattern or design in color instead of white, that is, an illuminated discharge print, it is preferable to apply, simultaneously with the destruction of the ground color, a dyestuff which is either resistant to re-

duction and is itself a dye for the fabric or one which can be reversibly oxidized after being vatted to the leuco form. In general, it is the vat dyes which are used for illumination since these dyestuffs are capable of being reversibly oxidized after being vatted. The vat dyestuffs are applied to the fabric mixed in with the discharge paste and the resulting paste applied in any pattern desired. The vat dyestuffs, however, must be sufficiently solubilized in the discharge paste so that they can penetrate the fabric properly and will give, on subsequent treatment, even and permanent colorations. To solubilize the vat dyes properly, the discharge paste must be alkaline in reaction since the vat dyes can not be adequately solubilized in a medium of acid reaction. Thus, when discharge printing textile materials, such as fabrics, which have been dyed with azo dyes having the characteristics heretofore mentioned, satisfactory white discharges may only be obtained with discharge agents of acid reaction and satisfactory illuminated discharge prints only with discharge agents of alkaline reaction. In the latter case, that is, in the preparation of illuminated discharge prints, alkaline discharge agents may frequently be employed even though they do not discharge the azo background color to a pure white. This is so because the illuminating vat color may frequently mask the off-white color of the discharge after the vat dye is oxidized to the colored form from the colorless leuco form. If the illuminating color is of a sufficiently dark shade, or the off-white shade of the discharge is light enough so as not to affect the illuminating color objectionably, the illuminated discharge print obtained by employing an alkaline discharging agent may often be acceptable. But the production of both white and colored discharges in a single operation employing an alkaline discharging agent could not be satisfactorily effected.

We have now discovered that both white and illuminated discharge prints may be obtained in a single operation with alkaline discharging agents on textile materials dyed with azo dyes obtained by diazotizing an amino compound of the following general formula:



wherein the halogen may be Br, Cl, F or I, and coupling said diazotized amino compound with

a coupling component comprising a substituted di-hydroxyalkyl-amino compound of the following general formula:



wherein R is a hydroxyalkyl group containing at least two carbon atoms, R' is an alkyl group, and X may be H, alkyl, O-alkyl or O-alkylene-OH. By employing azo dyestuffs of this group for the dyeing of textile materials made of or containing organic derivatives of cellulose, such as cellulose acetate, or synthetic linear polyamide condensation products, such as nylon, or other textile materials, it is possible to obtain these materials dyed with background colors in many valuable shades of blue, depending upon the particular components coupled, and to obtain white, and colored illuminated discharge prints on such materials by discharging the background color with alkaline discharging agents.

As examples of suitable alkaline discharging agents which may be employed in our process there may be mentioned sodium sulfoxylate formaldehyde and the sulfoxylate formaldehydes of calcium, barium, magnesium or strontium.

The substituted di-hydroxyalkyl-amino coupling components which may be used in the preparation of dyestuffs which may be discharged in accordance with our invention are compounds such as, for example, 2-di-hydroxyethyl-amino-4-acetylaminio-anisole, 2-di-hydroxypropyl-amino-4-propionylaminio-anisole, 2-di-( $\beta$ - $\gamma$ -hydroxypropyl)-4-acetylaminio-anisole, 2-dihydroxyethyl-amino-4-acetylaminio-phenetole, 2-dihydroxypropyl-amino-4-acetylaminio-phenetole, 2-di-hydroxyethyl-amino-4-acetylaminio-toluene, 2-di-hydroxyethyl-amino-4-acetylaminio-hydroxyethyl-phenol and other substituted amino compounds.

The dyes may be formed in substance by the usual diazotization methods and the material may be dyed directly in a bath containing the desired amount of dyestuff dispersed therein by means of a suitable detergent or dispersing agent.

In some instances, the material which is to be dyed may be based with the amino compound and the diazotization and coupling carried out on the material itself. The amino compound may be applied to the material in the form of dispersions or by bath or mechanical impregnation methods, such as padding or printing. After the amino compound has been applied to the material, it may be diazotized in the usual manner using sodium nitrite and sulfuric or hydrochloric acid. It is preferable that the diazotization be carried out at a low temperature, preferably below 20° C., and it may be carried out on a winch or jig or other suitable device for working the material. The coupling reaction may then be carried out by entering the treated material in a bath containing the coupling component. Thus, the material can be entered into a cold coupling bath which may then be heated, or the material can be entered into a bath already heated to about the desired coupling temperature. When the coupling is completed, the dyed material is scoured, rinsed and dried.

In formulating the discharge paste the alkaline discharge agent and the vat dye in the reduced form are mixed with a suitable thickening agent such as gum arabic, gum tragacanth, Brit-

ish gum or any of the commercially prepared gums, and swelling agents or penetrants for the material are added. Such swelling agents, in the case of cellulose acetate materials, are the thiocyanates of sodium and potassium and the penetrants may be liquids such as ethyl alcohol, glycol, thio-diglycol, etc.

The discharge paste may be applied to the fabric by means of embossed or engraved rollers, by stencil, or with blocks, or by other suitable means and the fabric can then be dried by passing through a drying tower or over heated cans or drums.

The portion of the fabric to be discharged to a white color is printed with a discharge paste composition free of the vat color while that portion which is to be illuminated is printed with a discharge paste having the desired vat color incorporated therein. By selecting the proper combination of rollers, stencils, etc., a print having two, three or even more colors may be prepared. Since an alkaline discharge agent is employed on both the area to be discharged to a white color and on the area to be illuminated, the pattern can be so chosen that the respective colored and white portions are in close contact and even in overlapping relationship without any danger of undesirable chemical reactions taking place between the respective areas, with the consequent formation of degraded material in which the pattern is poorly defined. The latter was a disadvantage which resulted, when employing an acid and an alkaline discharging agent in different portions of the pattern which were in fairly close contact since this causes the edges of the patterns to creep and destroys the sharpness and clarity of the resulting print. In addition, the fact that acid discharging agents are not present is especially advantageous when producing discharge patterns on mixed fabrics containing yarns of regenerated cellulose, since the strength of such yarns is adversely affected by the action of many discharging agents which are acid in reaction.

After drying, the printed fabric is passed through an ager so that the background color will be acted upon by the discharging agent in the paste and the color destroyed. The continuous ager or cottage ager may be used and the ageing is generally carried out at about 98° C. to 100° C. for a period of time sufficient to discharge the azo dye. This period may be from 10 to 20 minutes depending on the type of fabric, the particular dyestuffs used and the depth of shade. The fabric is then washed to remove the decomposition products as completely as possible and to wash out the alkaline solubilizing agent so that the insoluble leuco vat dye is precipitated. The vat dye may then be oxidized from the leuco form by exposure to air or by an oxidizing bath. After a final wash with water the fabric is dried.

While our invention is applicable to the discharge printing of various textile materials dyed with the class of dyes heretofore described, it is of particular importance with respect to fabrics or other textile material made of or containing yarns or filaments of silk, wool, organic derivatives of cellulose, such as cellulose esters and cellulose ethers, and textile materials comprising synthetic linear polyamide condensation products, such as nylon. Examples of cellulose esters are cellulose acetate, cellulose propionate, cellulose butyrate, and mixed esters such as cellulose acetate-propionate and cellulose acetate-butyrate.

ate, while examples of cellulose ethers are ethyl cellulose and benzyl cellulose. Mixed materials containing two or more of the aforementioned textile materials together with other textile materials such as regenerated cellulose may likewise be discharge printed in accordance with our invention.

In order further to illustrate our invention but without being limited thereto the following examples are given:

*Example I*

A cellulose acetate fabric is dyed in a medium blue shade with 2% of 2'-cyano-4'-nitro-6'-bromobenzene-azo-2-di-hydroxyethyl-amino-4-acetyl-amino-anisole. The fabric is then printed in a suitable pattern with a discharge paste made up as follows:

| Parts by weight                  |    |
|----------------------------------|----|
| Sodium sulphoxylate formaldehyde | 10 |
| Sodium thiocyanate               | 10 |
| Supertex gum                     | 45 |
| Water                            | 35 |

The printed fabric is then dried and aged in the rapid ager for 14 minutes at 100° C. The reduction products are removed by treating the fabric for 2 minutes in a 2 gram per liter solution of NaOH and the fabric is washed, rinsed and dried. A sharp white design on a medium blue background is obtained.

*Example II*

A cellulose acetate fabric is dyed in a light blue shade with 1% of 2'-cyano-4'-nitro-6'-bromobenzene-azo-2-di-hydroxyethylamino-4-acetyl-amino-anisole. The fabric is then printed in a suitable three-color pattern to yield white, green and red portions with the following discharge pastes:

For the white effect:

| Parts by weight                  |    |
|----------------------------------|----|
| Sodium sulphoxylate formaldehyde | 6  |
| Sodium thiocyanate               | 6  |
| Gum tragacanth paste             | 50 |
| Water                            | 38 |

For the green effect:

| Parts by weight                                                                 |    |
|---------------------------------------------------------------------------------|----|
| Sodium sulphoxylate formaldehyde                                                | 4  |
| Sodium thiocyanate                                                              | 4  |
| Soda ash                                                                        | 4  |
| Supertex gum                                                                    | 50 |
| Water                                                                           | 32 |
| Ponsol Jade Green (Color Index 1101)                                            | 3  |
| Ponsol Flavone GC (a vat dye)                                                   | 8  |
| Indanthrene Golden Yellow GK (Schultz Farbstofftabellen, 7th, vol. 2, page 130) | 4  |

For the red effect:

| Parts by weight                  |    |
|----------------------------------|----|
| Sodium sulphoxylate formaldehyde | 6  |
| Sodium thiocyanate               | 6  |
| Caustic soda                     | 4  |
| Sulphanthrene Pink F (a vat dye) | 15 |
| Supertex gum                     | 45 |
| Water                            | 24 |

The printed fabric is then dried and aged in a rapid ager for 14 minutes at 100° C. The fabric is then washed in 2 gram per liter caustic soda cold for 2 minutes and the vat colors are then oxidized by a treatment in 5 gram per liter sodium perborate and 1 gram per liter soap for 2 minutes at 50° C. The fabric is then rinsed and dried.

It is to be understood that the foregoing detailed description is given merely by way of ill-

ustration and that many variations may be made therein without departing from the spirit of our invention.

Having described our invention, what we desire to secure by Letters Patent is:

1. Process for the production of white discharge printing effects upon a textile material dyed with an azo dyestuff formed by diazotizing an amino compound of the following general formula:



and coupling said diazotized amino compound with a di-hydroxyalkylamino compound having the following formula:



wherein R is a hydroxyalkyl group containing at least 2 carbon atoms, R' is an alkyl group and X is a member of the group consisting of hydrogen, alkyl, O-alkyl and O-alkylene-OH, which comprises applying to said dyed material in a predetermined pattern a discharge paste comprising a sulfoxylate formaldehyde discharge agent having an alkaline reaction.

2. Process for the production of discharge printing effects upon a textile material dyed with an azo dyestuff formed by diazotizing an amino compound of the following general formula:



and coupling said diazotized amino compound with a di-hydroxyalkylamino compound having the following formula:



wherein R is a hydroxyalkyl group containing at least 2 carbon atoms, R' is an alkyl group and X is a member of the group consisting of hydrogen, alkyl, O-alkyl and O-alkylene-OH, to obtain a multicolored pattern having both white and illuminated areas, which comprises applying to said dyed material in a predetermined pattern a plurality of discharge paste compositions, each comprising a sulfoxylate formaldehyde discharge agent having an alkaline reaction and all but one of said compositions having a vat dye in the leuco form incorporated therein.

3. Process for the production of white discharge printing effects upon a textile material comprising an organic derivative of cellulose dyed with an azo dyestuff formed by diazotizing an amino compound of the following general formula:



and coupling said diazotized amino compound with a di-hydroxyalkylamino compound having the following formula:



wherein R is a hydroxyalkyl group containing at least 2 carbon atoms, R' is an alkyl group and X is a member of the group consisting of hydrogen, alkyl, O-alkyl and O-alkylene-OH, which comprises applying to said dyed material in a predetermined pattern a discharge paste comprising a sulfoxylate formaldehyde discharge agent having an alkaline reaction.

4. Process for the production of discharge printing effects upon a textile material comprising an organic derivative of cellulose dyed with an azo dyestuff formed by diazotizing an amino compound of the following general formula:



and coupling said diazotized amino compound with a di-hydroxyalkylamino compound having the following formula:



wherein R is a hydroxyalkyl group containing at least 2 carbon atoms, R' is an alkyl group and X is a member of the group consisting of hydrogen, alkyl, O-alkyl and O-alkylene-OH, to obtain a multicolored pattern having both white and illuminated areas, which comprises applying to said dyed material in a predetermined pattern a plurality of discharge paste compositions, each comprising a sulfoxylate formaldehyde discharge agent having an alkaline reaction and all but one of said compositions having a vat dye in the leuco form incorporated therein.

5. Process for the production of white discharge printing effects upon a textile material comprising cellulose acetate dyed with an azo dyestuff formed by diazotizing an amino compound of the following general formula:



and coupling said diazotized amino compound with a di-hydroxyalkylamino compound having the following formula:



wherein R is a hydroxyalkyl group containing at least 2 carbon atoms, R' is an alkyl group and X is a member of the group consisting of hydrogen, alkyl, O-alkyl and O-alkylene-OH, which

comprises applying to said dyed material in a predetermined pattern a discharge paste comprising a sulfoxylate formaldehyde discharge agent having an alkaline reaction.

5. Process for the production of discharge printing effects upon a textile material comprising cellulose acetate dyed with an azo dyestuff formed by diazotizing an amino compound of the following general formula:



and coupling said diazotized amino compound with a di-hydroxyalkylamino compound having the following formula:



25 wherein R is a hydroxyalkyl group containing at least 2 carbon atoms, R' is an alkyl group and X is a member of the group consisting of hydrogen, alkyl, O-alkyl and O-alkylene-OH, to obtain a multicolored pattern having both white and illuminated areas, which comprises applying to said dyed material in a predetermined pattern a plurality of discharge paste compositions, each comprising a sulfoxylate formaldehyde discharge agent having an alkaline reaction and all but one of said compositions having a vat dye in the leuco form incorporated therein.

7. Process for the production of white discharge printing effects upon a textile material dyed with a dyestuff prepared by diazotizing 2-cyano-4-nitro-6-brom-aniline and coupling said diazotized amine with 2-di-hydroxyethyl-amino-4-acetyl-amino-anisole, which comprises applying to said dyed material in a predetermined pattern a discharge paste comprising a sulfoxylate formaldehyde discharge agent having an alkaline reaction.

8. Process for the production of white discharge printing effects upon a textile material comprising cellulose acetate dyed with a dyestuff prepared by diazotizing 2-cyano-4-nitro-6-brom-aniline and coupling said diazotized amine with 2-di-hydroxyethyl-amino-4-acetyl-amino-anisole, which comprises applying to said dyed material in a predetermined pattern a discharge paste comprising a sulfoxylate formaldehyde discharge agent having an alkaline reaction.

9. Process for the production of discharge printing effects upon a textile material dyed with a dyestuff prepared by diazotizing 2-cyano-4-nitro-6-brom-aniline and coupling said diazotized amine with 2-di-hydroxyethyl-amino-4-acetyl-amino-anisole to obtain a multicolored discharge pattern having both white and illuminated areas on the background, which comprises applying to said dyed material in a predetermined pattern a plurality of discharge paste compositions, each comprising a sulfoxylate formaldehyde discharge agent having an alkaline reaction and all but one of said compositions having a vat dye in the leuco form incorporated therein.

10. Process for the production of discharge printing effects upon a textile material comprising an organic derivative of cellulose dyed with a dyestuff prepared by diazotizing 2-cyano-4-nitro-6-brom-aniline and coupling said diazo-

tized amine with 2-di-hydroxyethyl-amino-4-acetyl-amino-anisole to obtain a multicolored discharge pattern having both white and illuminated areas on the background, which comprises applying to said dyed material in a predetermined pattern a plurality of discharge paste compositions, each comprising a sulfoxylate formaldehyde discharge agent having an alkaline reaction and all but one of said compositions having a vat dye in the leuco form incorporated therein.

11. Process for the production of discharge printing effects upon a textile material comprising cellulose acetate dyed with a dyestuff prepared by diazotizing 2-cyano-4-nitro-6-brom-aniline and coupling said diazotized amine with 2-dihydroxyethyl-amino-4-acetyl-amino-anisole to obtain a multicolored discharge pattern having both white and illuminated areas on the background, which comprises applying to said dyed material in a predetermined pattern a plurality of discharge paste compositions, each comprising a sulfoxylate formaldehyde discharge agent having an alkaline reaction and all but one of said compositions having a vat dye in the leuco form incorporated therein.

12. Process for the production of discharge printing effects upon a textile material comprising cellulose acetate dyed with a dyestuff prepared by diazotizing 2-cyano-4-nitro-6-brom-aniline and coupling said diazotized amine with 2-dihydroxyethyl-amino-4-acetyl-amino-anisole, which comprises locally applying to said dyed material in a predetermined pattern a plurality of discharge paste compositions, each comprising sodium sulfoxylate formaldehyde and all but one of said compositions having a vat dye in the leuco form incorporated therein.

13. Process for the production of white dis-

- charge printing effects upon a textile material comprising cellulose acetate dyed with a dyestuff prepared by diazotizing 2-cyano-4-nitro-6-brom-aniline and coupling said diazotized amine with 2-dihydroxyethyl-amino-4-acetyl-amino-anisole, which comprises applying to said dyed material in a predetermined pattern a discharge paste comprising 10 parts by weight of sodium sulfoxylate formaldehyde, 10 parts of sodium thiocyanate, 10 parts of a thickening agent and 35 parts of water.
14. Process for the production of discharge printing effects upon a textile material comprising cellulose acetate dyed with a dyestuff prepared by diazotizing 2-cyano-4-nitro-6-brom-aniline and coupling said diazotized amine with 2-dihydroxyethyl-amino-4-acetyl-amino-anisole, to obtain a multicolored discharge pattern having both white and illuminated areas in the background, which comprises applying to said dyed material in a predetermined pattern a plurality of discharge paste compositions, one of said discharge paste compositions comprising 6 parts by weight of sodium sulfoxylate formaldehyde, 6 parts of sodium thiocyanate, 50 parts of a thickening agent and 38 parts of water, another comprising 4 parts by weight of sodium sulfoxylate formaldehyde, 4 parts of sodium thiocyanate, 4 parts of soda ash, 41 parts of a thickening agent, 3 parts of Ponsol Jade Green, 8 parts of Ponsol Flavone GC, 4 parts of Indanthrene Golden Yellow GK and 32 parts of water, and another 6 parts by weight of sodium sulfoxylate formaldehyde, 6 parts of sodium thiocyanate, 4 parts of caustic soda, 15 parts Sulphanthrene pink F, 45 parts of a thickening agent and 24 parts of water.

GEORGE W. SEYMOUR.

VICTOR S. SALVIN.